

## UNITED STATES PATENT OFFICE

EDGAR ARTHUR ASHCROFT, OF WAYE HOUSE, NEAR ASHBURTON, ENGLAND

## EXTRACTION OF TIN FROM ORES OR MATERIALS CONTAINING TIN

No Drawing. Application filed May 5, 1928, Serial No. 275,560, and in Great Britain July 7, 1927.

This invention relates to improvements in the metallurgy of tin bearing ores or materials whereby the valuable contents thereof may be extracted in a more convenient and economical manner than heretofore.

It is useful in the treatment of ores, concentrates, slags, alloys, residues or tin-containing materials of almost any kind. Particularly it is useful in the extraction of tin from ores or concentrates containing tin in the form of cassiterite such as the well known "lode tin" or "alluvial" ores which occur throughout the world, or of any form of concentrates therefrom.

The present invention is characterized in that during or after the reduction of the tin bearing minerals or compounds—for instance cassiterite—or tin slag compounds—by any suitable reducing agent—I employ a catalyzing or carrying salt and another metal—which I will call a collecting metal and which is preferably the metal nickel—into which under the conditions stated the tin will enter and alloy therewith, leaving the body of ore or gangue matter nearly or quite free from tin. It is further characterized by the recovery of the tin from its alloy with the collecting metal in any useful forms or combinations and by any of several appropriate means, all as hereinafter explained.

As "catalyzing or carrying salt" I may employ any of a large number of compounds which are capable of acting in the manner explained, particularly ferrous chloride zinc chloride or ammonium chloride. In fact I may define the term "carrying salt" as any salt capable of forming volatile compounds with tin.

The said salt may be employed in comparatively small quantities for instance 0.5 per cent to 5 per cent of the weight of material under treatment. The collecting metal may be employed in quantities suitable to form alloys of the desired composition with the tin present in the charge. The most economical and efficient proportions of both or either may be readily found for each material to be treated by calculation and by a few preliminary tests or trials.

The several methods of carrying out this

invention as far as the reduction of the tin is concerned, may be substantially similar to those described in my co-pending application Serial No. 275,267, filed May 4th, 1928, or I may employ carbonaceous or gaseous reducing agents in lieu of metal powders in known ways or any suitable combination of one with the other method of reduction. I may employ any convenient apparatus and dispositions of the respective materials—  
55 "tin bearing material" "reducing agent" "catalyzing or carrying salt" and "collecting metal" and may vary the same without departing from the spirit of my invention. For instance I may employ nickel containers,  
60 nickel plates or nickel shot graded small pellets or powders mixed with the charge under treatment and then separate out the alloy of tin and nickel so produced by means of any known or suitable recovery process, for  
65 instance magnetic or gravity concentration. A good method is to employ graded nickel powder or small pellets of say minus 50 plus 100 mesh. After treatment the alloy may then be separated from the gangue matter  
70 by simple screening, the other materials having been all passed through the 100 mesh or other selected screen previous to treatment.

To illustrate the principles of my invention I will describe some of my early experiments wherein I employed zinc chloride as the "catalyzing or carrying salt" and a nickel containing vessel as the "collecting metal" with iron powder as the reducing agent, but  
85 I do not limit myself to these materials, dispositions or forms of procedure.

## Experiment No. 1

An ore of "lode tin" taken from a Cornish mine was selected carrying 1.2 per cent Sn as cassiterite in a matrix of granite with a few per cent of pyrites. To emphasize the results and make more accurate determinations this ore was enriched to 6.93 per cent Sn  
90 by the addition of a Nigerian tin concentrate containing 58.5 per cent Sn as cassiterite in the ratio of 1 of concentrate to 9 of Cornish ore.

The charge mixture consisted of 45 grams  
95

of Cornish ore and 5 grams of cassiterite with 5 grams iron powder all intimately mixed and ground to pass 100 mesh sieve.

With the charge was also intimately mixed 2.0 grams anhydrous zinc chloride.

The whole was placed in a nickel crucible with cover weighing 70.35 grams and heated for 20 minutes to between 700° and 800° centigrade and allowed to cool without admission of air. The whole had lost barely 2 grams in weight. On opening the crucible the charge was found to have uniformly shrunk and caked to a soft but coherent sinter and could be removed from the crucible in one piece by merely tipping it out and afterwards pulverized with great ease.

The charge contained only a trace of tin. The crucible had increased in weight by 3.7 grams and on assay was found to contain practically the whole of the tin originally in the ore and concentrate namely, 3.47 grams. The crucible was clean and with metallic lustre on inside surface which however was blistered all over. The inner blistered surface assayed as high as 28 per cent Sn and the rest of the crucible in reducing amounts at progressively greater depths from the inner surface.

#### Experiment No. 2

The same procedure as in Experiment No. 1 was repeated but omitting the enrichment of the Cornish ore by the Nigerian cassiterite. The quantities were Cornish ore 75 grams, iron powder 5 grams. Zinc chloride—one piece placed in centre of charge in this case 2.0 grams, crucible and cover 67.8 grams.

The charge was treated as in No. 1 and—after cooling—the ore contained no tin and the crucible—quite clean and of metallic surface—had increased by 1.8 grams in weight. This was found to include the whole of the 0.9 gram of tin originally contained in and now taken from the ore and some iron arsenic and sulphur.

The experiment repeated a number of times with fresh charges of ore but using the same crucible resulted in a continual increase of weight of the crucible by absorption of all the tin in each successive fresh charge in approximately quantitative increments until the crucible had become quite a rich alloy.

The hereinbefore described experiments were repeated omitting the "catalyzing or carrying salt" all other conditions being as before. It was found that some tin was transferred from the charge to the nickel crucible under these conditions but not to anything like the same extent. The charges after treatment usually contained about  $\frac{2}{3}$  to  $\frac{1}{2}$  of the original tin content.

These experiments were repeated using ferrous chloride and again using ammonium chloride as catalyzing or carrying salt with

equally good results in each case. They were also repeated using charcoal and again using anthracite as reducing agents and again using iron containers and employing a nickel collecting metal in the form of graded small pellets and as powders all with complete success.

It was found that both sulphur and arsenic will enter the alloys if present in the ore under treatment and that when these impurities are present in any considerable amounts a previous roast whereby arsenic and sulphur are removed in known ways improves the quality of the alloys of tin and nickel produced as aforesaid and also reduces the amounts of reagents required. Some iron usually enters the alloy together with the tin, the amount depending both on the temperature and period of the heating and on the proportion of the iron present. Such iron is not usually detrimental in such alloys and is sometimes of advantage.

I will state two typical examples of the production of such alloys using iron chloride and carbonaceous reducing agents in the presence of iron oxide but I do not limit myself to these examples or to the precise form of the reactions or to the materials or the proportions of materials indicated. These examples are based on my actual experiments.

#### Example No. 1

It is desired to reduce the tin oxide in a good grade ore or a low grade cassiterite concentrate, putting the tin into alloy with both nickel and iron so as to make an alloy which can be separated from the gangue matter magnetically and which shall contain a comparatively small amount of nickel per unit of tin this being desirable for economic reasons in the subsequent recovery of both metals.

A suitable mixture is approximately as follows:

|                                                                                           | Pounds |
|-------------------------------------------------------------------------------------------|--------|
| Ore (or concentrate) containing 6 per cent Sn                                             | 110    |
| FeCl <sub>2</sub> ·2H <sub>2</sub> O (or anhydrous in proportion)                         | 200    |
| Fe <sub>2</sub> (HO) <sub>3</sub> (or anhydrous in proportion)                            | 2      |
| Coal (or charcoal)                                                                        | 11     |
| Nickel (added as metal pellets or as metal powder or as oxide or hydrated oxide) as metal | 115    |
|                                                                                           | 6      |
|                                                                                           | 20     |
| Total charge                                                                              | 239    |

But mixtures richer in tin and/or iron and poorer in nickel or vice versa may be employed if preferred for any reason.

The nickel is here indicated as applied in the form of metal in a divided state. It may however be applied as oxide or hydroxide just as it is precipitated from its solutions or after calcining or reducing to a metal

powder, in which case additional coal or other reducing agent may be used to reduce the oxide to metal.

After heating to about 700 to 900 degrees centigrade for one hour or less during which time small quantities of  $H_2O$  and  $CO_2$  with  $CO$  and a little  $HCl$  will distill off, all the tin and nickel and most of the iron present will be found in association as a highly magnetic alloy of approximately the following composition:

|    | Per cent |
|----|----------|
| Ni | 51.75    |
| Fe | 16.95    |
| Sn | 31.3     |
|    | 100.0    |

and the weight approximately 38 lbs. of alloy.

This alloy may be completely and easily separated from the gangue by magnetic means.

If the nickel employed is nickel which has been reduced from its hydrated oxide (as for instance on further treatment of the alloy for recovery of its tin) and is converted into tiny pellets of -50+100 screen size for instance by the well known Mond nickel carbonyl reaction or otherwise, these pellets will absorb the iron and the tin and the alloy so formed may be completely separated from gangue matter by simple screening, provided that the original charge of ore, coal and iron chloride and oxide have all been previously pulverized to pass the selected screen size. Or if the nickel is employed as an ungraded powder (reduced from its oxide in situ or otherwise prepared and added to the charge) such fine portions of alloy as cannot be screened free from gangue may be readily separated magnetically.

If less iron is required in the alloy the mixture may be modified as follows:

|                                                                   | Pounds |
|-------------------------------------------------------------------|--------|
| Ore or concentrate (containing 6 per cent Sn)                     | 200    |
| $FeCl_2 \cdot 2H_2O$ { or anhydrous salts } acting as catalysts   | 1.0    |
| $Fe_2(HO)_6$ only in this case.                                   | 0.5    |
| Coal                                                              | 3      |
| Nickel (as pellets or as powder or as oxide or hydroxide) (metal) | 20     |
| Total charge                                                      | 224.5  |

The composition of the resulting alloy will then be approximately:

|    | Per cent |
|----|----------|
| Ni | 62.0     |
| Sn | 37.0     |
| Fe | 1.0      |
|    | 100.0    |

and the weight approximately 33 lbs.

If the charge has not been overheated this

alloy is also easily separated by screening or by magnetic means.

Alloys with low iron and low nickel content are somewhat less though still appreciably magnetic up to about 65 to 75 per cent of tin.

#### Example No. 2

A mixture suitable in case of a rich ore or concentrate is as follows:

|                                   | Pounds |
|-----------------------------------|--------|
| Concentrate (60% Sn)              | 200    |
| $Fe_2(HO)_6$ or anhydrous         | 5      |
| $FeCl_2 \cdot 2H_2O$ or anhydrous | 10     |
| Coal                              | 30     |
| Nickel (metal)                    | 200    |
|                                   | 445    |

The resulting alloy will weigh and assay as follows:

|             | Pounds | Per cent |
|-------------|--------|----------|
| Tin         | 120    | 36.6     |
| Nickel      | 200    | 61.0     |
| Iron (app.) | 8      | 2.4      |
| Total       | 328    | 100.0    |

The temperature of reduction should not exceed in any case 800 to 900 degrees centigrade and air should be excluded whilst heating the charges.

After the tin has been collected into the collecting metal I may recover it therefrom in any known or suitable way.

Or I may melt the alloys and cast them into anodes and use such anodes in an electrolytic bath of suitable composition whereby I may obtain tin and nickel plated out separately onto sheet metal cathodes in known or suitable ways whilst the anodes are dissolved and serve to depolarize the baths so that a minimum of electric energy is required therefor and the baths are refurnished by the solution of metals at the anodes.

As far as I am aware the reaction hereinbefore described whereby the tin will transfer itself from a distance through a considerable thickness of charge into a collecting metal without contact therewith and with that metal still in the solid phase are all novel and hitherto unknown.

I cannot yet offer any definite explanation of the precise mechanism of these reactions which require further study, but in general it may be conceived that tin in the form of tin chloride is vapourized in small amounts and that the catalyzing or carrying salt also in the form of a vapour bath of a very high degree of mobility transfers the tin chloride vapour rapidly into contact with the exposed surfaces of the collecting metal which in turn at the temperatures employed decomposes it and absorbs the tin like a sponge whilst chlorine is set free and combines with additional metal in the charge. It is probable

that at the temperature employed there is sufficient balance of free energy—due to the considerable energy of formation of the nickel alloy—to enable these reactions to take 5 place.

The herein described process is of great technical value in the recovery and metallurgy of tin as it provides a ready and inexpensive method of concentrating and reducing to metal the tin values in almost any tin bearing material of high or low grade.

In the case especially of low or intermediate grade ores or products and in the case of tin bearing slags and of complex tin bearing 10 ores containing other metals and sulphur, the tin may be recovered at only a fraction of the cost of existing methods and many such materials now of no commercial value may by its use be profitably employed for 15 the production of tin.

Throughout this specification the terms ore or material are intended whenever applicable by the context to include any ore, concentrate, product, slag, residue or other material 20 from which tin is to be extracted. The terms furnace or retort are intended to include horizontal, sloping or vertical retorts; muffle or open furnaces, with or without rabbling devices; revolving furnaces, kilns, tunnel ovens, pallet chains of Dwight Lloyds sintering type; or any form of heating apparatus the heat for which may be supplied by solid, liquid or gaseous fuel or by electricity.

35 **What I claim is:—**

1. In the extraction of tin from a mass of tin-bearing material, mixing with the mass a carrying salt and a collecting metal, and heating the mass to cause the tin to alloy 40 with the collecting metal.

2. In the extraction of tin from a mass of tin-bearing material, reducing the tin to metallic form, mixing with the mass a carrying salt and a collecting metal after reduction 45 has commenced, heating the mass to cause the tin to alloy with the collecting metal, and subsequently separating the tin from said collecting metal.

3. In the extraction of the tin from a mass of tin-bearing material, mixing with the mass a metal chloride and a collecting metal, and heating the mass to cause the tin to alloy 50 with the collecting metal.

4. In the extraction of tin from a mass of tin-bearing material, mixing with the mass a carrying salt and nickel, and heating the mass to cause the tin to alloy with the nickel.

5. In the extraction of tin from a mass of tin-bearing material, mixing with the mass a metal chloride and nickel, and heating the mass to cause the tin to alloy with the nickel.

6. In the extraction of tin from a mass of tin-bearing material, mixing with the mass ammonium chloride and nickel, and heating 65

the mass to cause the tin to alloy with the nickel, substantially as described.

In testimony whereof I have signed my name to this specification.

EDGAR ARTHUR ASHCROFT. 70

75

80

85

90

95

100

105

110

115

120

125

130